# EUROPEAN PATENT SPECIFICATION

(11) **EP 0 008 853 B1**
(45) Date of publication and mention of the grant of the patent: **04.08.1982**
(21) Application number: 79301311.1
(22) Date of filing: 06.07.1979
(51) Int. Cl.: D01F 6/38, D01D 5/10

(54) **Process for melt spinning acrylonitrile polymer fibres**
Schmelzspinnverfahren zur Herstellung von Polyacrylnitrilfasern
Procédé pour le filage à l'état fondu de fibres de polymères d'acrylonitrile

(30) Priority: 30.08.1978 US 938196; 30.08.1978 US 938197; 30.08.1978 US 938202
(43) Date of publication of application: 19.03.1980
(73) Proprietor: AMERICAN CYANAMID COMPANY, Wayne New Jersey 06904 (US)
(72) Inventor: Pfeiffer, Ronald E., Pensacola, Florida (US); Peacher, Stanley E., Milton, Florida (US); Roberts, Robert W., New London, Missouri (US)
(74) Representative: Allam, Peter Clerk

## Description

This invention relates to a process for melt-spinning fiber-forming polymers at an increased production rate per spinnerette. More particularly, this invention relates to such a process wherein a spinnerette with more orifices per given area than previously possible is employed. The greater density of orifices may arise from closer crowding of conventional sized orifices and associated counterbores, from close crowding of smaller orifices and associated counterbores, or by employing multiple orifices per counterbore.

In conventional melt-spinning of fibers, a fiber-forming polymer is heated to a temperature at which it melts, is extruded through a spinnerette plate to form filaments which rapidly cool to become solid, and the resulting filaments are then further processed to provide the desired fiber. The spinnerette plate that is employed in such processing must contain capillaries to provide the desired filaments while satisfying two additional requirements. The capillaries must be of such dimensions as to satisfy back-pressure requirements and must be sufficiently spaced from one another as to prevent premature contact between the emerging fibers that would result in sticking together or fusion of filaments with one another. To satisfy the back-pressure requirements, the capillaries are provided with counterbores of sufficient diameter and depth.

Recent developments in the field of fiber spinning, especially acrylic fibers, has led to the development of fusion melts which can be extruded through a spinnerette plate to provide filaments. These fusion melts comprise a homogeneous composition of a fiber-forming polymer and a melt assistant therefor. The melt assistant is a material which enables the polymer to form a melt at a temperature below which the polymer would normally melt or decompose and becomes intimately associated with the molten polymer so that a single phase melt results. The melt assistant must be used in proper proportions with the polymer to provide the single-phase fusion melt. If a low boiling melt assistant is used the melt assistant in proper amounts and the polymer often must be heated at pressures above atmospheric pressure to provide the fusion melt. Since the temperature at which the fusion melt forms is above the boiling point of the melt assistant at atmospheric pressure, consequently super-atmospheric pressures are necessary to keep the melt assistant in the system. Such fusion melts have been effectively spun into fiber using spinnerette plates similar to those employed in conventional melt-spinning.

Because of the requirement for adequate spacing of the capillaries in spinnerette plates used for melt-spinning to prevent premature contact between the nascent filaments which would result in their sticking together, the number of capillaries that can be provided in a given spinnerette plate is greatly restricted. As a result, production capacity of a spinnerette with a given surface area is limited and usually large tow bundles can only be produced by combining the outputs from a series of spinnerettes. This, in turn, requires costly installations of additional spinnerettes, specially designed conduits and spin packs to ensure an even distribution of the melt to all spinning holes, provision of space for installation, and further power consumption to operate the increased number of spinnerettes.

There exists, therefore, the need for processes for providing fiber by melt spinning which enables the productivity of spinnerettes to be increased. Such provision would fulfill a long-felt need and constitute a significant advance in the art.

In accordance with the present invention there is provided a process for melt-spinning an acrylonitrile polymer fiber which comprises providing a homogeneous fusion melt of a fiber-forming acrylonitrile polymer and water at a temperature above the boiling point of water at atmospheric pressure and at a temperature and pressure which maintains water in single phase with said polymer and extruding said fusion melt through a spinnerette assembly containing a spinnerette plate having an orifice density of at least 18 per square centimeter directly into a steam-pressurized solidification zone maintained under conditions such that the rate of release of water from the nascent extrudate avoids deformation thereof.

In a preferred embodiment, the spinnerette plate has orifices of 60 to 160 microns and the acrylonitrile polymer has a kinematic molecular weight in the range of 30,000 to 60,000.

In another preferred embodiment, the spinnerette plate has a plurality of counterbores within each of which are contained at least 3 capillaries.

Another preferred embodiment includes the step of stretching the nascent extrudate while it remains within said solidification zone to provide desirable textile properties. In such embodiment, it is generally preferred to conduct such stretching in at least two stages with the first stage being conducted at a stretch ratio less than that of the subsequent stage.

The present invention, by employing a fusion melt of an acrylonitrile fiber-forming polymer and water at a temperature above the boiling point of water at atmospheric pressure and at a temperature and pressure that maintains water and the polymer in a single phase and by extruding the fusion melt directly into a steam-pressurized solidification zone maintained under conditions such that the rate of release of water from the nascent extrudate avoids deformation thereof, provides filamentary extrudates which do not stick together as they emerge from the spinnerette orifices. Since the filaments have no tendency to stick together as they emerge from the spinnerette, the orifices of the spinnerette plate can be located closer together and more orifices can be provided in the spinnerette plate. As a result, the productivity of a spinnerette can be greatly increased without negatively affecting the quality of the resulting fiber.

The present invention also enables the use of orifices of reduced cross-section relative to those conventionally employed in melt-spinning. As a result an even greater number of orifices can be present in the spinnerette plate. In order to overcome back-pressure difficulties that would arise with the orifices of narrow cross-section, the process of the present invention in this embodiment employs fiber-forming polymers of lower molecular weight than conventionally employed. Unexpectedly, the fiber obtained possessses good fiber properties in spite of the low molecular weight of the fiber-forming fiber. It is believed these good fiber properties are the result of processing steps employed.

The spinnerette plate used in the process of the present invention contains a much greater density of orifices per unit area than do conventional spinnerette plates used in melt spinning by conventional procedures. Typically, prior art melt-spinning spinnerette plates have a density of 5-10 orifices per square centimeter at most. In the process of the present invention the spinnerette plate contains at least about 18 orifices per square centimeter, preferably at least 25, 50 or more per square centimeter. This enables the process of the present invention to provide a substantial increase in productivity from a given spinnerette. Since processing of the melt is under conditions which lead to nascent extrudates which do not stick together or deform, the higher density of spinnerette orifices is possible.

Conventional, melt-spinning spinnerette plates have orifices of about 200--400 microns or larger diameter at their exits ends. The process of the present invention may employ orifice of such conventional diameters but preferably uses orifices in the range of about 60₋160 microns diameter at their exit ends. This provision not only allows a greater number of orifices to be positioned in the spinnerette plate to increase productivity but also enables finer denier fiber to be provided at a given stretch ratio.

In another preferred embodiment, the spinnerette plate of the present invention contains a number of capillaries located within each counterbore. The counterbores are necessary to enable the spinnerette plate to operate at a suitable level of back-pressure. The spinnerette plate as a whole will contain a substantially greater number of capillaries than the prior art spinnerette plates associated with melt spinning because the problem of sticking together of nascent extrudates is eliminated. Increased productivity is provided by increasing the density of capillaries in the spinnerette plate and the number of capillaries in each counterbore beyond the operative limits of conventional melt-spinning spinnerette plates which have restrictions as to hole density imposed by fusing of individual filaments.

It is possible to provide larger counterbores than are normally associated with a capillary and provide numerous capillaries therein although this has often been found to be unnecessary. It is preferable to provide a pattern of counterbores more closely spaced than those in the prior art spinnerette plates for melt spinning in a pattern providing uniform extrusion of the spinning melt through the spinnerette plate. The combination of more closely spaced counterbores with a plurality of capillaries within each counterbore gives rise to a substantial increase in the total number of capillaries for a given spinnerette surface, and hence in the productivity of the spinnerette.

In carrying out the process of the present invention, it is necessary to provide a homogeneous fusion melt of a fiber-forming acrylonitrile polymer that can form a fusion melt with water at a temperature above the boiling point of water at atmospheric pressure and at a pressure and temperature sufficient to maintain water and the polymer in a single fluid phase. Polymers falling into this category are known in the art. Preferred acrylonitrile fiber-forming polymers are those having kinematic molecular weights ranging from about 30,000 to 60,000, as defined below. The fusion melt is prepared at a temperature above the boiling point at atmospheric pressure of water and eventually reaches a temperature and pressure sufficient to maintain water and the polymer in a single, fluid phase.

The homogeneous fusion melt thus provided is extruded through the spinnerette plate of the present invention directly into a steam-pressurized solidification zone that controls the rate of release of water from the nascent filaments so that deformation thereof is avoided and the process is able to provide filaments which solidify without sticking together one with another in spite of the close proximity of adjacent capillaries. The extruded filaments may be processed according to conventional procedures to provide desirable filamentary materials which may have application in textile and other applications.

The pressurized solidification zone used in the process of the present invention is a critical feature of the process. If this pressurized solidification zone is omitted, water is so rapidly released from the nascent filaments which would emerge into atmospheric conditions that the filaments would become inflated or deformed and interfere with neighboring filaments and necessitate reduction in the number of operative spinnerette capillaries which would defeat the object of the invention. On the other hand, by employing the pressurized solidification zone operating at suitable steam pressure, the rate of release of water can be controlled as the nascent filaments solidify so that foaming and deformation thereof is avoided and optimum stretching is possible.

The particular pressure of steam will vary widely depending upon the polymer employed, the spinning temperature employed and the like. The useful values for given systems are those values which minimize or avoid foaming or other forms of deformation of the filaments and provide optimum stretching. These values can readily be determined for any given system of polymer and water taking into account the teachings herein given.

A particularly preferred embodiment of the process of the present invention is drawing the nascent extrudate while it remains in the steam-pressurized solidification zone. Such drawing can be accomplished in one or more stretches and can eliminate any subsequent drawing normally required for fiber orientation. It is particularly preferred to conduct drawing in two stages with the stretch ratio of the second stage being larger than that of the first stage. It is also preferred to relax the drawn fiber in steam generally under conditions which provide from about 20% to 35% filament shrinkage.

The invention is more fully illustrated in the examples which follow wherein all parts and percentages are by weight unless otherwise specified.

Kinematic average molecular weight (Mₖ) is obtained from the following relationship: wherein µ is the average effluent time (t) in seconds for a solution of 1 gram of the polymer in 100 milliliters of 53 weight percent aqueous sodium thiocyanate solvent at 40°C multiplied by the viscometer factor and A is the solution factor derived from a polymer of known molecular weight and in the present case is equal to 3,500.

### Comparative example A

A single phase fusion melt was prepared using a copolymer containing 89.3% acrylonitrile and 10.7% methyl methacrylate and having an intrinsic viscosity of 1.52. This fusion melt was extruded through a spinnerette having 1266 capillaries each of diameter 200 microns. Each of the capillaries was centered in a counter bore of 2.0 millimeters in diameter and dispersed at a spacing of 4.0 millimeters center-to-center in the spinnerette plate, the density of orifices being 5 per square centimeter of spinnerette plate extrusion surface. Extrusion was conducted at 176°C and the extrudate issued directly into a solidification zone maintained at 25 psig i.e. a gauge pressure of 171244 N/m² (130°C) with saturated steam. The extrudate was subjected to a first stage of stretching at a stretch ratio of 3.2 and a second stage of stretching at a stretch ratio of 13.6 while the extrudate remained in the solidification zone. The stretch ratio was the speed of the extrudate take-up relative to the linear flow of fusion melt through the spinnerette. The total stretch ratio obtained was 43.5. The extrudate, representing a bundle of filaments, which emerged from the solidification zone was relaxed in saturated steam at a pressure of 18 psig i.e. a gauge pressure of 123296 N/m² (124°C) during which a shrinkage of 285 occurred. The fiber before relaxation was 5.4 denier/filament and 7.2 denier/filament after relaxation. Relaxed fiber properties were as follows:

### Example 1

Following the procedure of Comparative Example A in every material detail except for the spinnerette plate employed, an additional extrusion run was made. In this example, a smaller spinnerette plate was employed but it contained 2937 orifices each of 200 micron diameter centered in counterbores of 1.0 millimeter diameter, the density of orifices being 67 per square centimeter of spinnerette plate extrusion surface.

Extrusion was conducted without any sticking together of individual filaments and fiber identical to that obtained in Comparative Example A was obtained.

### Comparative example B

The procedure of Example 1 was repeated in every material detail except that a polypropylene melt free of melt assistant and designated as fiber grade having a melt index of 3 (Trademark Rexene PP-3153) was employed and extrusion was conducted at 260-280°C directly into air. The extrudates stuck together as they emerged from the spinnerette and the desired individual filaments could not be obtained.

Example 1 compared to Comparative Example A shows that the process of the present invention provides desirable fiber using closely spaced orifices. Comparative Example B compared to Example 1 shows that other melt-spinning compositions are not effectively processed using closely spaced orifices.

### Examples 2-5

Again following the procedure of Example 1, a series of runs were made in which the spacing of the orifices in the spinnerette plate was varied. In each instance fiber of substantially the same properties as those of the fiber of Example 1 was obtained. Example numbers and spinnerette plate details are given below:

### Example 6

A fusion melt of 14% water and 86% of an acrylonitrile polymer of the following composition was prepared:

This polymer had a kinematic molecular weight value of 40,000.

The fusion melt was spun through a spinnerette plate having the following characteristics:

The extrusion temperature was 170°C and extrusion was directly into a steam-pressurized solidification zone maintained at 13 pounds per square inch gauge i.e. a gauge pressure of 89047 N/m^{2.} The extrudates were stretched at a stretch ratio of 4.2 in a first stage and 9.8 in a second stage, dried at 138°C and steam relaxed at 116°C. No filament breakage or sticking occurred. The fiber obtained had the following properties:

### Comparative example C

Following the procedure of Example 6 in every material detail, an additional run was made using a polypropylene melt free of melt assistant and designated as fiber grade having a melt index of 3 (Trademark Rexene PP-3153) in place of the fusion melt of example. Extrusion was conducted at 260-280°C directly into air. The extrudates stuck together as they emerged from the spinnerette and the desired individual filaments could not be obtained.

### Examples 7-11

Again following the procedure of Example 6 in every material detail except for the spinnerette plate, a series of runs were made using spinnerettes of the characteristics given in Table 11 which also indicates the example number. In each instance, no filament breakage or sticking occurred and the fiber obtained had properties substantially similar to those of the fiber of Example 6.

### Example 12

The process of Example 6 was again repeated in every material detail except that the polymer employed was a copolymer of 94% acrylonitrile and 6 methyl acrylate having a kinematic molecular weight of 48,000. No filament breakage or sticking occurred during extrusion and the filter obtained had substantially the same properties as those of Example 6.

### Example 13

A fusion melt of 1 5% water and 85% of the acrylonitrile polymer of the following composition was prepared at autogeneous pressure and 170°C:

The fusion melt was spun at 170°C through a spinnerette assembly having orifice characteristics as follows:

The extrusion was directly into a solidification zone pressurized with saturated steam at 15 pounds per square inch i.e. 102746 N/m². The extruded filaments were stretched in a first stage at a stretch ratio of 3.8 and in a second stage at 6.7 for a total stretch of 25.5x. The filaments were dried at 138°C and relaxed in steam at 116°C. Fiber of about 12 denier per filament was obtained having the following properties:

No sticking together of the filaments occurred and continuous processing was accomplished.

### Comparative example D

Using the spinnerette assembly described in Example 13, a melt polypropylene (Rexene Grade PP 3153) of fiber grade having a melt index of 3 dg/min was prepared at 260°C and extruded into static air at 25°C. The melt emerging from the union of the individual filaments issuing from single capillaries. Thus, filaments of the desired denier were not obtained using this spinnerette plate design.

### Example 14

The procedure of Example 13 was again followed with the following exceptions: The polymer had a kinematic molecular weight value of 40,000 and the spinnerette assembly had the following characteristics:

Continuous spinning was conducted with no sticking together or fusion of the individual filaments and fiber of substantially the same properties as obtained in Example 13 was obtained.

When the polypropylene melt described in Comparative Example D was extruded, extensive fusion of the individual filaments occurred and it was not possible to provide the desired filament denier.

### Examples 15-17

Following the procedure of Example 13, a number of runs were made using spinnerette assemblies of different design in each run as shown in Table III which also gives the example number. In each instance, continuous spinning was effected wtih no sticking together of the individual filaments.

## Claims

1. A process for melt-spinning an acrylonitrile polymer fiber by providing a homogeneous fusion melt of a fiber-forming acrylonitrile polymer and water at a temperature above the boiling point of water at atmospheric pressure and at a temperature and pressure which maintains water in single phase with said polymer, and extruding said fusion melt through a spinnerette assembly containing a spinnerette plate directly into a steam-pressurized solidification zone maintained under conditions such that the rate of release of water from the nascent extrudate avoids deformation thereof, characterized in that said spinnerette plate has an orifice density of at least 18 per square centimeter of spinnerette plate extrusion surface.

2. The process of Claim 1 wherein the spinnerette plate has orifices of a diameter of 60 to 160 microns and the acrylonitrile polymer has a kinematic molecular weight in the range of 30,000 to 60,000.

3. The process of Claim 1 or Claim 2, wherein the spinnerette plate has a plurality of counterbores within each of which are contained at least 3 capillaries.

4. The process of any preceding claim, including the step of stretching the nascent extrudate while it remains within said solidification zone.

5. The process of Claim 4, wherein said stretching is conducted in at least two stages, the first stage being at a stretch ratio less than that of the subsequent stage.

6. The process of Claim 4 or Claim 5, wherein the drawn fiber is relaxed in steam under conditions to provide from about 20-35% filament shrinkage.

## Revendications

1. Procédé de filage à l'état fondu d'une fibre de polymère d'acrylonitrile en fournissant une masse fondue homogène d'un polymère d'acrylonitrile formant des fibres et d'eau à une température supérieure au point d'ebullution de l'eau à la pression atmosphérique et à une temperature et une pression qui maintiennent l'eau en une phase unique avec ledit polymère et en extrudant ladite masse fondue à travers un ensemble formant filière contenant une plaque de filière directement dans une zone de solidification sous pression de vapeur d'eau maintenue dans des conditions telles que la vitesse de libération de l'eau à partir de l'extrudat naissant évite sa déformation, caracterise en ce que ladite plaque filière a une densité d'orifices d'au moins 18/cm² de la surface d'extrusion de la plaque filière.

2. Procédé selon la revendication 1, dans lequel la plaque filière a des orifices de 60 à 160 _{jU}m de diamètre et le polymère d'acrylonitrile a un poids moléculaire cinématique compris dans la gamme de 30 000 à 60 000.

3. Procédé selon la revendication 1 ou 2, dans lequel la plaque filière a plusieurs contre-trous contenant chacun au moins trois capillaires.

4. Procédé selon l'une quelconque des revendications précédentes, comprenant un stade d'étirage de l'extrudat naissant tandis qu'il demeure dans ladite zone de solidification.

5. Procédé selon la revendication 4, dans lequel ledit étirage est effectué en au moins deux stades, le rapport d'étirage dans le premier stade étant inferieur à celui du stade suivant.

6. Procede selon la revendication 4 ou 5, dans lequel la fibre étirée est relachée dans de la vapeur d'eau dans des conditions telles que l'on obtienne un retrait du filament d'environ 20 à 35%.

## Patentansprüche

1. Verfahren zum Schmelzspinnen von Acrylnitrilpolymerfasern, bei dem man eine homogene Fusionsschmelze aus einem faserbildenden Acrylnitrilpolymeren und Wasser bereitet, und zwar bei einer Temperatur oberhalb des Siedepunktes des Wassers bei Atmosphärendruck und unter Temperatur- und Druckbedingungen, welche das Wasser in einer einzigen Phase mit dem Polymeren halten, worauf man die Fusionsschmelze durch eine Spinndüsenanordnung mit einer Spinndüsenplatte extrudiert, und zwar direkt in eine mit Dampf unter Druck gesetzte Erstarrungszone, welche unter solchen Bedingungen gehalten wird, dass die Geschwindigkeit der Freisetzung des Wassers aus dem austretenden Extrudat eine Deformation desselben verhindert, dadurch gekennzeichnet, dass die besagte Spinndüsenplatte eine Öffnungsdichte von mindestens 18 Öffnungen/cm² der Extrudierfläche der Spinndüsenplatte aufweist.

2. Verfahren nach Anspruch 1, wobei die Spinndüsenplatte Öffnungen mit einem Durchmesser von 60 bis 160 Mikron aufweist und wobei das Acrylnitrilpolymere ein kinematisches Molekulargewicht im Bereich von 30 000 bis 60 000 aufweist.

3. Verfahren nach Anspruch 1 oder 2, wobei die Spinndüsenplatte eine Vielzahl von Senkbohrungen aufweist, deren jede mindestens 3 Kapillaren enthält.

4. Verfahren nach einem der vorhergehenden Ansprüche, einschliesslich des Verfahrensschrittes, bei dem das austretende Extrudat gereckt wird, während es sich noch in der Erstarrungszone befindet.

5. Verfahren nach Anspruch 4, wobei das Recken in mindestens zwei Stufen durchgeführt wird, wobei das Reckverhältnis in der ersten Stufe geringer ist als in der nachfolgenden Stufe.

6. Verfahren nach Anspruch 4 oder 5, wobei die gereckten Fasern in Dampf entspannt werden, unter Bedingungen, welche zu einer Filamentschrumpfung von etwa 20 bis 35% führen.
